

1

2,981,686

## METAL WORKING LUBRICANTS

Thomas E. Reamer, El Cerrito, Calif., assignor to Shell Oil Company, a corporation of Delaware

No Drawing. Filed Oct. 30, 1958, Ser. No. 770,592

10 Claims. (Cl. 252—33.6)

This invention relates to aqueous base metal-working lubricating compositions. More particularly, it relates to a water-base metal cutting fluid.

It is well known in the art that water base fluids possess good cooling properties for processing metals, but that they lack the lubricity and extreme pressure properties of oil base lubricants and usually cause corrosion. On the other hand, oil base lubricants are inferior coolants and are costly.

The art discloses various means of imparting rust inhibiting and extreme pressure properties to water base metal-working lubricants, but with little success. Among the materials commonly used for this purpose are water-soluble non-ionic compounds, such as alkyl phenolethylene oxide reaction products, tallow, fatty acids, soaps, such as sodium or potassium oleate or sulfonate, in combination with water-soluble alkali metal compounds and mixtures thereof, such as the nitrites, phosphates, carbonates, or chromates, e.g., mixtures of sodium nitrite and sodium phosphate, or mixtures of sodium nitrite and sodium carbonate. Water-oil emulsions additionally present a dermatitis and stability problem upon use and are generally undesirable because of their opaqueness thus making it difficult to observe the machining process.

It is an object of this invention to provide a cutting fluid having both good cooling and good lubricating properties. Another object of the invention is to provide a non-corrosive aqueous cutting solution. Still another object of the invention is to provide a stable, non-corrosive, aqueous cutting composition free of ingredients capable of causing dermatitis infections. Another object of the invention is to provide a multi-functional metal working lubricant useful at high speeds, heavy loads, high pressures and high temperatures.

The above and other objects are attained in accordance with the present invention by an aqueous medium, such as water containing from about 0.5% to about 15%, preferably from 2% to 10% by weight each of (1) a water-soluble normal alkali metal salt of a polymercaptop-(thio-)carboxylic acid having the general formula  $R(S_yR_1-COOH)_x$  wherein R and R<sub>1</sub> can be the same or different alkylene groups of from 1 to 6 and preferably from 1 to 4 carbon atoms such as methylene, ethylene or butylene groups, x is an integer of from 2 to 4, and y is an integer of 1 to 2; (2) an alkanolamine, such as mono-, di- or triethanolamine, mono-, di-, or tripropanolamine, etc., or the like; and (3) a water-soluble hetero copolymeric alkylene glycol, ether or ester thereof, wherein the different oxyalkylene units are substantially randomly distributed throughout the entire polyoxyalkylene chain. The final water base fluid should have a pH between 8 and 11, preferably from about 9 to about 10.

The combination of the above three essential additives function in a particular manner and produce an outstanding metal working fluid. The polymercaptopcarboxylates function as extreme pressure and load carrying agents, the alkanolamines inhibit corrosion without producing any undesirable side effects, which is not true of alkali

2

metal nitrites which form unstable solutions in combination with polymercaptopcarboxylates. The water-soluble hetero copolymer improves the antifrictional properties of compositions of the present invention, particularly under slow sliding conditions. On the other hand, other non-ionic polymeric compounds such as alkyl phenol-ethylene oxide reaction products, block copolymers of dissimilar alkylene oxides and their derivatives such as are commercially available under the trade name of "Pluronics" and the like produce undesirable frictional problems, foaming, instability and the like.

The alkylene polymercaptopcarboxylic acids are prepared by reacting an aliphatic mercapto carboxylic acid with an aliphatic carbonyl compound such as an aliphatic aldehyde. Methods of preparing such acids are described by Ritter et al., JACS 74, 5576 (1952), or Holmberg et al., Ann 353, 123 (1907). Among the mercapto acids are included mercaptoacetic acid, alpha or beta-mercaptopropionic acids, alpha,beta-dimercaptopropionic acid, alpha-mercaptopbutyric acid and the like. The organic carbonyl compounds include aldehydes such as formaldehyde, acetaldehyde, butyraldehyde, glyoxal, or ketones such as acetone, butanone, etc.

The water-soluble neutral polyalkali metal salts of an alkylene polymercaptopcarboxylic acid include di- or tetra-sodium, lithium or potassium salt of methylene bis(mercaptoproacetic acid), ethylene bis(mercaptoproacetic acid), methylene bis(mercaptopropionic acid), methylene bis(mercaptopropane acid), methyl bis(mercaptoproacetic acid), ethylene tetrakis(mercaptoproacetic acid), ethylene tetrakis(mercaptopropionic acid), and mixtures thereof.

The water-miscible hetero-copolymer polyalkylene oxide fluids enhance the load carrying properties of the composition of the present invention. The above oxides are hetero-copolymers of dissimilar alkylene oxides such as copolymer ethylene oxide and 1,2-propylene oxide [poly(oxyethylene-1,2-oxypropylene)glycol], as well as monoethers and monoesters thereof, preferably at oxide ratios of from 75:25 to 10:90 ethylene oxide to 1,2-propylene oxide, and molecular weight from about 250 to about 1500.

By a ratio of from 75:25 to 10:90 is meant that, in the formation of copolymer the amount of 1,2-propylene oxide is from  $\frac{1}{3}$  to 9 times the amount of ethylene oxide present, by weight, the parts or proportion of the 1,2-propylene oxide being given last. These materials are described in U.S. Patents 2,425,755 and 2,425,845. The copolymer diols may be employed in a modified form as the monoethers or monoesters of monohydric alcohols or monobasic acids with the diols. The alcohols preferably have from 1 to about 10 carbon atoms, while the mono-carboxylic acids preferably have from 1 to 12 carbon atoms.

The alkanolamines which are used in compositions of this invention include mono-, di- and triethanolamine, propanolamine, N,N-dimethylisopropanolamine, and mixtures thereof.

The following compositions are representative of the invention, which can be used neat or diluted with from 1 to 10 parts of water, as metal-working lubricants for cutting, drilling and the like. The proportions are given in percentages by weight.

## Composition A

|                                                                                                           | Percent |
|-----------------------------------------------------------------------------------------------------------|---------|
| 65 Disodium methylene bis(mercaptopacetate)<br>[CH <sub>2</sub> (S—CH <sub>2</sub> —COONa) <sub>2</sub> ] | 2       |
| 55 Hetero-copolymer of ethylene oxide-1,2-propylene oxide (75/25) having a viscosity of 450 at 100° F.    | 10      |
| 60 Triethanolamine                                                                                        | 2       |
| 70 Water                                                                                                  | Balance |

## Composition B

|                                                                                                                                       |         |
|---------------------------------------------------------------------------------------------------------------------------------------|---------|
| Tetrasodium salt of ethylene tetrakis(mercaptopoacetic acid) [C <sub>2</sub> H <sub>4</sub> (S—CH <sub>2</sub> —COONa) <sub>4</sub> ] | 2       |
| Hetero-copolymer of ethylene oxide-1,2-propylene oxide (75/25) having a viscosity of 1400 at 100° F.                                  | 10      |
| Triethanolamine                                                                                                                       | 2       |
| Water                                                                                                                                 | Balance |

## Composition C

|                                                                                                      |         |
|------------------------------------------------------------------------------------------------------|---------|
| Disodium salt of methylene bis(dimercaptopoacetic acid)                                              | 6       |
| Hetero-copolymer of ethylene oxide-1,2-propylene oxide (75/25) having a viscosity of 1400 at 100° F. | 10      |
| Dimethylisopropanolamine                                                                             | 2       |
| Sodium mercaptobenzothiazole                                                                         | 0.1     |
| Water                                                                                                | Balance |

## Composition D

|                                                                                                       |         |
|-------------------------------------------------------------------------------------------------------|---------|
| Tetrapotassium salt of ethylene tetrakis(mercaptopoacetic acid)                                       | 4       |
| Hetero-copolymer of ethylene oxide-1,2-propylene oxide (75/25), having a viscosity of 1400 at 100° F. | 10      |
| Diethanolamine                                                                                        | 4       |
| Sodium mercaptobenzothiazole                                                                          | 1       |
| Dimethyl silicone polymer                                                                             | 0.001   |
| Water                                                                                                 | Balance |

## Composition E

|                                                                                                     |         |
|-----------------------------------------------------------------------------------------------------|---------|
| Dipotassium salt of methylene bis(mercaptopoacetic acid)                                            | 2       |
| Hetero-copolymer of ethylene oxide-1,2-propylene oxide (75/25) having a viscosity of 450 at 100° F. | 10      |
| Triethanolamine                                                                                     | 2       |
| Water                                                                                               | Balance |

The outstanding properties of compositions of this invention are demonstrated by results obtained from subjecting them to the following tests:

(1) Four-ball machine tests as described in the Journal of the Institute of Petroleum Technology, pages 206-229, April 1946.

(2) Drilling test: The compositions were used in drilling deep 1" holes in AISI 4340 steel at 1440 r.p.m. and compared with a reference water base cutting fluid (X), the reference fluid being rated as 100%.

Compositions A-E in the four-ball test gave average weld loads of between 600 and 1000 kg., and these compositions gave values of from 300 to 800% above the reference fluid (X). The substitution of other salts of sulfur-containing carboxylic acids for the polyalkali metal mercaptopolycarboxylates used in compositions of this invention such as sodium mercaptoacetate or sodium dibutylthiocarbamate gave much lower weld loads in the four-ball machine, around 200-300. Also, the substitution of other types of non-ionic compounds for the heteropolymer used in Compositions A-E, such as a block copolymer of ethylene oxide and propylene oxide available commercially under the trade name "Pluronic L64" (Wyandotte Chemical Company) or an alkylphenol-ethylene oxide condensation product, caused excessive foaming, whereas compositions (A-E) of the present invention are non-foaming.

Compositions of this invention may contain additional additives, such as water-soluble corrosion inhibitor, e.g., sodium mercaptobenzothiazole, anti-foaming agents such as silicone polymer, perfuming agents, and dyes. The compositions may be applied with excellent results to general cutting operations where cooling and lubricating of the tool and work piece under adverse conditions are encountered. Metals machined with the aid of fluids of

this invention have good surface finish, are free from rust and the cutting tool life is excellent.

I claim as my invention:

1. An aqueous metal-working lubricant comprising a major amount of water and from about 0.5% to 15% each of (1) a water-soluble normal alkali metal salt of an alkylene poly(mercaptopoalkylene carboxylic acid), said compound having from 1 to 4 carboxyl groups in the molecule and the alkylene radical being selected from the group of methylene, ethylene and butylene radicals, (2) a water-soluble hetero-copolymer of a mixture of randomly distributed ethylene and propylene oxides in the molecular ratio of from 75:25 to 10:90, respectively, having a molecular weight of from about 250 to about 1500, and (3) a water-soluble alkanolamine.
2. An aqueous metal-working lubricant comprising a major amount of water and from about 2% to about 10% each of (1) a water-soluble neutral dialkali metal salt of an alkylene bis(mercaptopoalkylene carboxylic acid), the alkylene radical being selected from the group of methylene, ethylene and butylene radicals, (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.
3. An aqueous metal-working lubricant comprising a major amount of water and from about 2% to about 10% each of (1) a water-soluble neutral tetraalkali metal salt of an alkylene tetrakis(mercaptopoalkylene carboxylic acid), the alkylene radical being selected from the group of methylene, ethylene and butylene radicals, (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.
4. An aqueous metal-working lubricant comprising a major amount of water and from about 2% to about 10% each of (1) a water-soluble neutral disodium metal salt of an alkylene bis(mercaptopoalkylene carboxylic acid), the alkylene radical being selected from the group of methylene, ethylene and butylene radicals, (2) a water-soluble hetero-copolymer of ethylene oxide and 1,2-propylene glycol in the ratios of from 75:25 to 10:90 respectively and having a molecular weight of from about 250 to about 1500 and (3) a water-soluble ethanolamine.
5. An aqueous metal-working lubricant comprising a major amount of water and from about 2% to about 10% each of (1) a water-soluble neutral tetrasodium metal salt of an alkylene tetrakis(mercaptopoalkylene carboxylic acid), the alkylene radical being selected from the group of methylene, ethylene and butylene radicals, (2) a water-soluble hetero-copolymer of ethylene oxide and 1,2-propylene glycol in the ratios of from 75:25 to 10:90 respectively and having a molecular weight of from about 250 to about 1500, and (3) a water-soluble ethanolamine.
6. An aqueous metal-working lubricant comprising a major amount of water and from about 2% to about 10% each of (1) disodium salt of methylene bis(mercaptopoacetic acid), (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.
7. The composition of claim 6 containing from 0.01 to 1% of sodium mercaptobenzothiazole.
8. An aqueous metal-working lubricant comprising a major amount of water and from about 2% to about 10% each of (1) tetrasodium salt of ethylene tetrakis(mercaptopoacetic acid), (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.
9. An aqueous metal-working lubricant comprising a

major amount of water and from about 2% to about 10% each of (1) dipotassium salt of methylene bis(mercaptopropionic acid), (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.

10. An aqueous metal-working lubricant comprising a major amount of water and from about 2% to about 10% each of (1) tetrapotassium salt of ethylene tetrakis(thiopropionic acid), (2) a water-soluble hetero-copolymer of ethylene oxide and 1,2-propylene glycol in the ratios of from 75:25 to 10:90 respectively and having a molecular weight of from about 250 to about 1500 and (3) a water-soluble alkanolamine.

15

## References Cited in the file of this patent

## UNITED STATES PATENTS

|   |           |                        |                |
|---|-----------|------------------------|----------------|
| 5 | 2,425,755 | Roberts et al. -----   | Aug. 19, 1947  |
|   | 2,425,845 | Toussaint et al. ----- | Aug. 19, 1947  |
|   | 2,449,992 | Gresham et al. -----   | Sept. 28, 1948 |
|   | 2,602,816 | Gregory et al. -----   | July 8, 1952   |
|   | 2,825,693 | Beaubien et al. -----  | Mar. 4, 1958   |

## FOREIGN PATENTS

|    |         |                     |              |
|----|---------|---------------------|--------------|
| 10 | 716,354 | Great Britain ----- | Oct. 6, 1954 |
|    | 721,526 | Great Britain ----- | Jan. 5, 1955 |